

May 27, 1952

R. E. STAUFFER ET AL  
HIGH-SPEED PHOTOGRAPHIC SILVER HALIDE EMULSIONS  
SUPERSENSITIZED WITH PALLADIUM SALTS  
Filed Aug. 31, 1948

2,598,079

FIG. 1.



A = RECIPROCITY CURVE FOR EMULSION SENSITIZED WITH POTASSIUM CHLOROAURATE AND SODIUM THIOCYANATE AND FINISHED TO SOMEWHAT BELOW OPTIMUM SPEED

B = RECIPROCITY CURVE FOR SAME EMULSION CONTAINING POTASSIUM CHLOROPALLADATE

FIG. 2.



C = RECIPROCITY CURVE FOR EMULSION SENSITIZED WITH POTASSIUM CHLOROAURATE AND SODIUM THIOCYANATE AND FINISHED TO OPTIMUM SPEED

D = RECIPROCITY CURVE FOR SAME EMULSION CONTAINING POTASSIUM CHLOROPALLADATE

ROBERT E. STAUFFER  
WILLIAM F. SMITH  
INVENTORS

BY  
A. M. Perrins  
Daniel J. Drayne  
ATTORNEYS

## UNITED STATES PATENT OFFICE

2,598,079

## HIGH-SPEED PHOTOGRAPHIC SILVER HALIDE EMULSIONS SUPERSENSITIZED WITH PALLADIUM SALTS

Robert E. Stauffer and William F. Smith, Rochester, N. Y., assignors to Eastman Kodak Company, Rochester, N. Y., a corporation of New Jersey

Application August 31, 1948, Serial No. 47,108

15 Claims. (Cl. 95—7)

1

This invention relates to high speed photographic silver halide emulsions supersensitized with palladium salts.

It is known that high speed photographic silver halide emulsions can be prepared by incorporating in the emulsions labile sulfur sensitizing bodies or gelatins and/or gold compounds. We have now found that such high speed emulsions can be supersensitized by adding to them a palladium salt. Thus, the emulsion can be brought to maximum sensitivity with the gold compound and then be rendered still more sensitive with the palladium salt, or the emulsion can be brought to a sensitivity short of the maximum sensitivity attainable with the gold compound and then be rendered more sensitive with the palladium salt. In addition, we have found that the palladium salts act as sensitizers for the low intensity portion of the reciprocity curve of such emulsions sensitized with gold compounds.

It is, accordingly, an object of our invention to provide new supersensitized high-speed photographic silver halide emulsions. A further object is to provide a process for preparing such emulsions. Other objects will become apparent hereinafter.

In accordance with our invention, we incorporate in a high-speed silver halide emulsion which is sensitized with at least one gold compound and/or at least one sulfur sensitizer, at least one palladium salt. The high-speed silver halide emulsions sensitized with at least one gold compound can be prepared by incorporating at least one gold compound in a photographic silver halide emulsion at any stage of the preparation of the emulsion or when the emulsion is completed, e. g. just before coating of the emulsion. The gold compound is advantageously employed in a concentration equal to not more than 0.015 per cent by moles of the silver halide in the emulsion, and in the case of gelatino-silver-bromide (including the so-called bromoiodide emulsions of which the majority of the halide is bromide, with a few per cent of iodide), the upper limit is advantageously 0.01 per cent by moles. Up to 0.015 per cent by moles of the silver halide in the emulsion, the amount of the gold compound can vary widely, as perceptible effects can be obtained with 0.0003 per cent or less. Advantageously, the lower limit is about 0.001 per cent by moles of the silver halide in the emulsion. We have found that from 0.003 per cent to about 0.005 per cent by moles is advantageously employed in practice, especially when the gold compound is incorporated in the emulsion during

2

the preparation of the emulsion, i. e. especially when the emulsion is digested in the presence of the gold compound.

The gold compounds can be added to the emulsions at any stage of the preparation of the emulsions, i. e. before or during precipitation of the silver halides, before or during the first digestion (ripening) of the emulsion, before or during the second digestion of the emulsion, or the gold compounds can be added to the emulsion just before coating the emulsion. The gold compounds are advantageously incorporated in the emulsions in the form of their solutions in a suitable solvent, e. g. water, methyl alcohol, ethyl alcohol, etc.

The gold compounds which we have found are most advantageously employed in preparing the high speed emulsions are the gold halides, such as auric chloride, or complex gold halides, such as potassium chloroaurate ( $KAuCl_4$ ) and sodium chloroaurate ( $NaAuCl_4$ ). However, gold compounds, such as auric sulfate, are practically as useful as the gold halides. Aurous, as well as auric compounds can be used. Complex gold salts, such as alkali metal aurous thiosulfates, alkali metal aurous sulfites (e. g. sodium or potassium aurous thiosulfate and sodium or potassium aurous sulfite), and a complex salt formed by the interaction of thiourea and auric chloride, are also suitable. Potassium chloroaurite, potassium bromoaurite, potassium iodoaurite, potassium auricyanide, potassium aurithiocyanate or the corresponding sodium, calcium, strontium, cadmium or gallium salts can also be used. Pyridinotrichloro-gold, ethylenediamine-bis-trichloro gold, diethyl-monobromo-gold and diethyl gold acetone and gold complexes with sulfur compounds such as are commonly present in gelatin, e. g. the gold thiosamine complexes, can also be used.

Sulfur sensitizers are advantageously also added to the emulsions. Gelatins normally contain certain sulfur compounds which act as sulfur sensitizers of photographic emulsions, but beneficial effects are obtained in accordance with our invention by adding sulfur sensitizers, i. e. sulfur compounds containing  $>C=S$  groups or  $—S—S—$  groups, e. g. thiourea, allyl isothiocyanate, thiosamine (allylthiourea), etc. Beneficial effects are also obtained by adding metal or ammonium thiocyanates, e. g. sodium, potassium, ammonium, calcium or cadmium thiocyanates, to the emulsion. Of course, thiocyanates containing cations which cations are known to have, in themselves, a deleterious effect on silver

halide emulsions should be avoided. Otherwise the beneficial effects of the thiocyanate would be partially nullified by the deleterious effect of the cation. Thus, iron thiocyanate should be avoided. One or more sulfur sensitizers can be employed, and one or more thiocyanates selected from the group consisting of metal and ammonium thiocyanates can be employed in conjunction with a sulfur sensitizer other than a thiocyanate containing a cation selected from the group consisting of metal and ammonium cations. The sulfur sensitizers are advantageously incorporated in the emulsions in the form of their solutions in a suitable solvent, such as water, methyl or ethyl alcohol.

The sulfur sensitizers can be incorporated in the emulsions at any stage of the preparation of the emulsion, e. g. during the precipitation of the silver halides, during the first digestion (ripening) or during the second digestion of the emulsion. When incorporating thiocyanates in the emulsions prior to washing the amount can vary widely. Advantageously, however, an amount of thiocyanate equal to from about 2 to about 15 per cent by moles of the silver halide in the emulsion is advantageously employed. If the thiocyanate or other sulfur sensitizer is not added until later in the preparation of the emulsion, e. g. after washing, it is advantageous to employ an amount equal to from about 0.1 to about 2.5 per cent by moles of the silver halide present in the emulsion in the case of metal and ammonium thiocyanates, and an amount equal to from about 0.006 to about 0.06 per cent by moles of the silver halide in the case of other sulfur sensitizers.

It is advantageous to digest, i. e. heat treat the emulsion with the gold compound with or without the sulfur sensitizer, at an appropriate temperature, e. g. at from 100 to 150° F. During digestion, i.e. the second digestion as contrasted with the first digestion or ripening, the pH of the emulsion is advantageously adjusted to the acid side of neutrality, e. g. between 5 and 7. Maintenance of the emulsion on the acid side of neutrality during coating of the emulsion is also advantageous.

The palladium salts which we employ in practicing our invention can be represented by the following general formulas:



wherein M represents a member selected from the group consisting of an alkali metal atom and an ammonium radical, and X represents a halogen atom selected from the group consisting of chlorine, bromine and iodine atoms. Typical of such palladium salts are: ammonium chloropalladate, potassium chloropalladate, sodium chloropalladate, ammonium chloropalladate, sodium chloropalladate, potassium bromopalladate, potassium iodopalladate, etc.

The palladium salts are advantageously added to the emulsion just before coating the emulsion, but can be added at any time to the finished emulsions. One or more of the palladium salts can be used. The palladium salts are advantageously incorporated in the emulsions in the form of their solutions in a suitable solvent, e. g. water, methyl alcohol, etc.

The palladium salts are advantageously employed in a concentration of from 0.015 to 0.2 per cent by moles of the silver halide in the emulsion. Usually from 0.3 to 0.15 per cent by moles produces the maximum supersensitizing effect.

The following examples will serve to illustrate further the manner of practicing our invention:

*Example 1*

A high speed photographic gelatino-silver bromide emulsion of the negative type sensitized with potassium chloroaurate (KAuCl<sub>4</sub>) and sodium thiocyanate was prepared and finished to somewhat below optimum speed. To separate batches of this emulsion were then added various palladium salts. The batches were coated on glass plates, the coated plates dried and then tested in a sensitometer, development being at 68° F. for 5 minutes in Eastman Kodak Company's "DK-50" developer. Results were as follows:

| Palladium salt, (percent by moles of silver halide in the emulsion) | Speed (1/i) | Gamma | Fog  |
|---------------------------------------------------------------------|-------------|-------|------|
| none                                                                | 18.5        | 0.82  | 0.02 |
| (NH <sub>4</sub> ) <sub>2</sub> PdCl <sub>6</sub> (0.05)            | 22.5        | 0.89  | 0.02 |
| (NH <sub>4</sub> ) <sub>2</sub> PdCl <sub>4</sub> (0.05)            | 24.0        | 0.85  | 0.02 |
| K <sub>2</sub> PdCl <sub>6</sub> (0.05)                             | 27.0        | 0.80  | 0.02 |

*Example 2*

A high speed photographic gelatino-silver bromide emulsion of the negative type sensitized with potassium chloroaurate (KAuCl<sub>4</sub>) and sodium thiocyanate was prepared and finished to optimum speed. Potassium chloropalladate was added to the emulsion. The emulsion was coated on a glass plate, the coated plate dried and then tested in a sensitometer, development being at 68° F. for 5 minutes in Eastman Kodak Company's "DK-50" developer. Results were as follows:

| Potassium Chloropalladate, (percent by moles of silver halide in the emulsion) | Speed (1/i) | Gamma | Fog  |
|--------------------------------------------------------------------------------|-------------|-------|------|
| none                                                                           | 29.0        | 0.80  | 0.03 |
| 0.05                                                                           | 38.0        | 0.79  | 0.03 |

The palladium salts act to sensitize the emulsions sensitized with the gold compounds, for the low-intensity portion of the reciprocity curve. For many purposes, such as astronomical and spectroscopic photography, it is useful to have photographic emulsions showing a low reciprocity failure at low intensities. The effect of the palladium salts in this respect is apparent from the curves in the accompany drawing. Fig. 1 shows reciprocity curves for the emulsion of Example 1 (with and without K<sub>2</sub>PdCl<sub>6</sub>) in which log I (meter candles) is plotted against log I<sub>t</sub> (meter candle seconds) (density=1.0+fog) in the manner customarily employed to illustrate reciprocity law failure (see The Theory of the Photographic Process, C. E. K. Mees, page 242, MacMillan Company, New York, 1942). Curve A represents the emulsion without the palladium salt and curve B represents the emulsion with the palladium salt. It will be observed that the emulsion containing the palladium salt shows distinctly lower reciprocity failure at low intensities than does the emulsion without the palladium salt, curve B curving upwards only at about 10 seconds, while curve A shows an upward slope at less than  $\frac{1}{10}$  second exposure. The ideal, of course, would be a straight-line curve throughout the entire range of exposures.

Fig. 2 shows reciprocity curves for the emulsions of Example 2, (with and without K<sub>2</sub>PdCl<sub>6</sub>) in which log I is plotted against log I<sub>t</sub> (den-

sity=1.0+fog) as in Fig. 1. Curve C in Fig. 2 represents the emulsion without the palladium salt and curve D represents the emulsion with palladium salt. It will be observed that the emulsion containing the palladium salt shows distinctly lower reciprocity failure especially at the lower intensities.

The emulsions prepared in accordance with our invention can be coated in the usual manner on supports such as glass, photographic film base, e. g. cellulose acetate type, photographic paper base, etc. Sensitizing dyes of all types can be employed to spectrally sensitize our new emulsions, e. g. erythrosin, Congo Red, any of the sensitizing cyanine dyes, any of the sensitizing merocyanine dyes (see United States Patent 2,078,233, dated April 27, 1937, for example), any of the sensitizing hemicyanine dyes (see United States Patent 2,166,736, dated July 18, 1939, for example) and of the sensitizing hemioxonol dyes (see United States Patent 2,165,339, dated July 11, 1939, for example), etc.

Our invention is directed primarily to the customarily employed photographic silver halide developing-out emulsions, e. g. silver chloride, silver chlorobromide, silver chlorobromoiodide, silver bromide and silver bromoiodide developing-out emulsions. A suitable gelatino-silver-halide emulsion is described, for example, by A. P. H. Trivelli and W. F. Smith, Phot. J. 79, 330 (1939). Such an emulsion can be prepared as follows:

In a container equipped with a temperature control was put a solution of the following composition:

A. potassium bromide ----- g. 825  
gelatin ----- g. 325  
water ----- cc. 8,500

and in another container was put a solution consisting of:

B. silver nitrate ----- g. 1,000  
water ----- cc. 10,000

Solution A was kept at a temperature of 70° C. and Solution B was put in a separatory funnel at a temperature of 72° C. Solution B was allowed to run, in 20 minutes, from the separatory funnel through a calibrated nozzle into solution A which was kept in constant motion during the precipitation of the silver halide. After precipitation of the silver halide, the resulting emulsion while being kept in constant motion was ripened for 20 minutes at 70° C. Then, the emulsion was cooled as quickly as possible to 45° C. and at this temperature, 1250 g. of washed gelatin were added to the emulsion. The emulsion was stirred for 20 minutes at 45° C. in order to dissolve the gelatin. After standing overnight in a cold storage room (10° C.), the emulsion was shredded and washed. It was then melted at a temperature of 42° C. The weight of the emulsion was brought to 31.5 kgs. by adding 500 g. of gelatin soaked in the required amount of distilled water. The emulsion was then finished at 60° C. to the desired speed, in the presence of one or more gold compounds and one or more sulfur sensitizers (see Examples 1 and 2).

The sensitization of photographic silver halide emulsions by means of gold compounds alone, or with sulfur sensitizers is well known in the art.

What we claim as our invention and desire to be secured by Letters Patent of the United States is:

1. A high speed photographic silver halide emulsion sensitized with at least one gold com-

ound in a concentration equal to from 0.0003 to 0.015% by moles of the silver halide in the emulsion, said emulsion containing as a supersensitizer, at least one palladium salt selected from the group consisting of palladium salts represented by the following general formulas:

$M_2PdX_6$  and  $M_2PdX_4$ ,

wherein M represents a member selected from the group consisting of an alkali metal atom and an ammonium radical, and X represents a halogen atom selected from the group consisting of chlorine, bromine and iodine atoms, the concentration of said palladium salt in the emulsion being equal to from 0.015 to 0.2% by moles of the silver halide in the emulsion.

2. A high speed photographic gelatino-silver-halide developing-out emulsion sensitized with at least one gold compound in a concentration equal to from 0.001 to 0.01% by moles of the silver halide in the emulsion, said emulsion containing as a supersensitizer at least one palladium salt selected from the group consisting of palladium salts represented by the following general formulas:

$M_2PdX_6$  and  $M_2PdX_4$ ,

wherein M represents a member selected from the group consisting of an alkali metal atom and an ammonium radical, and X represents a halogen atom selected from the group consisting of chlorine, bromine and iodine atoms, the concentration of said palladium salt in the emulsion being equal to from 0.015 to 0.2% by moles of the silver halide in the emulsion.

3. A high speed photographic gelatino-silver-halide developing-out emulsion sensitized with at least one gold salt selected from those represented by the following general formula:

$M'AuCl_4$ ,

wherein M' represents an alkali metal atom, said emulsion containing, as a supersensitizer, at least one palladium salt selected from those represented by the following general formula:

$M_2PdCl_6$

wherein M represents an alkali metal atom, the concentration of said gold salt being equal to from 0.001 to 0.01% by moles of the silver halide in the emulsion and the concentration of said palladium salt being equal to from 0.015 to 0.2% by moles of the silver halide in the emulsion.

4. A high speed photographic gelatino-silver-halide developing-out emulsion sensitized with potassium chloroaurate ( $KAuCl_4$ ) in a concentration equal to from 0.001 to 0.01% by moles of the silver halide in the emulsion, said emulsion containing, as a supersensitizer, potassium chloropalladate ( $K_2PdCl_6$ ) in a concentration equal to from 0.015 to 0.2% by moles of the silver halide in the emulsion.

5. A high speed photographic gelatino-silver-halide developing out emulsion sensitized with potassium chloroaurate ( $KAuCl_4$ ) in a concentration equal to from 0.001 to 0.01% by moles of the silver halide in the emulsion, said emulsion containing, as a supersensitizer, potassium chloropalladite ( $K_2PdCl_4$ ) in a concentration equal to from 0.015 to 0.2% by moles of the silver halide in the emulsion.

6. A high speed photographic gelatino-silver-halide developing-out emulsion sensitized with potassium chloroaurate ( $KAuCl_4$ ) in a concentration equal to from 0.001 to 0.01% by moles of

the silver halide in the emulsion, said emulsion containing as a supersensitizer, potassium bromopalladate ( $K_2PdBr_6$ ) in a concentration equal to from 0.015 to 0.2% by moles of the silver halide in the emulsion.

7. A high speed photographic gelatino-silver-halide developing-out emulsion sensitized with at least one gold compound in a concentration equal to from 0.0003 to 0.015% by moles of the silver halide in the emulsion, and at least one sulfur sensitizer, said emulsion containing, as a supersensitizer, at least one palladium salt selected from the group consisting of palladium salts represented by the following general formulas:



wherein M represents a member selected from the group consisting of an alkali metal atom and an ammonium radical, and X represents a halogen atom selected from the group consisting of chlorine, bromine and iodine atoms, the concentration of said palladium salt in the emulsion being equal to from 0.015 to 0.2% by moles of the silver halide in the emulsion..

8. A high speed photographic gelatino-silver-halide developing-out emulsion sensitized with at least one gold compound in a concentration equal to from 0.001 to 0.01% by moles of the silver halide in the emulsion, and at least one thiocyanate selected from the group consisting of alkali metal and ammonium thiocyanates in a concentration equal to from 0.1 to 2.5% by moles of the silver halide in the emulsion, said emulsion containing, as a supersensitizer, at least one palladium salt selected from the group consisting of palladium salts represented by the following general formulas:



wherein M represents a member selected from the group consisting of an alkali metal atom and an ammonium radical, and X represents a halogen atom selected from the group consisting of chlorine, bromine and iodine atoms, the concentration of said palladium salt in the emulsion being equal to from 0.015 to 0.2% by moles of the silver halide in the emulsion.

9. A high speed photographic gelatino-silver-halide developing-out emulsion sensitized with at least one gold salt selected from those represented by the following general formula:



wherein M' represents an alkali metal atom, in a concentration equal to from 0.001 to 0.01% by moles of the silver halide in the emulsion, and at least one thiocyanate selected from the group consisting of alkali metal and ammonium thiocyanates in a concentration equal to from 0.1 to 2.5% by moles of the silver halide in the emulsion, said emulsion containing, as a supersensitizer, at least one palladium salt selected from those represented by the following general formula:



wherein M represents an alkali metal atom, the concentration of said palladium salt in the emulsion being equal to from 0.03 to 0.15% by moles of the silver halide in the emulsion.

10. A high speed photographic gelatino-silver-halide developing-out emulsion sensitized with potassium chloroaurate ( $KAuCl_4$ ) in a concentration equal to from 0.001 to 0.01% by moles of the silver halide in the emulsion, and at least

one thiocyanate selected from the group consisting of alkali metal and ammonium thiocyanates in a concentration equal to from 0.1 to 2.5% by moles of the silver halide in the emulsion, said emulsion containing, as a supersensitizer, potassium chloropalladate ( $K_2PdCl_6$ ) in a concentration equal to from 0.03 to 0.15% by moles of the silver halide in the emulsion.

11. A high speed photographic gelatino-silver-halide developing-out emulsion sensitized with potassium chloroaurate ( $KAuCl_4$ ) in a concentration equal to from 0.001 to 0.01% by moles of the silver halide in the emulsion, and at least one thiocyanate selected from the group consisting of alkali metal and ammonium thiocyanates in a concentration equal to from 0.1 to 2.5% by moles of the silver halide in the emulsion, said emulsion containing, as a supersensitizer, potassium chloropalladite ( $K_2PdCl_4$ ) in a concentration equal to from 0.03 to 0.15% by moles of the silver halide in the emulsion.

12. A high speed photographic gelatino-silver-halide developing-out emulsion sensitized with potassium chloroaurate ( $KAuCl_4$ ) in a concentration equal to from 0.001 to 0.01% by moles of the silver halide in the emulsion, and at least one thiocyanate selected from the group consisting of alkali metal and ammonium thiocyanates in a concentration equal to from 0.1 to 2.5% by moles of the silver halide in the emulsion, said emulsion containing, as a supersensitizer, potassium bromopalladate ( $K_2PdBr_6$ ) in a concentration equal to from 0.03 to 0.15% by moles of the silver halide in the emulsion.

13. A process for preparing a high speed photographic silver halide emulsion comprising sensitizing the emulsion with at least one gold compound in a concentration equal to from 0.0003 to 0.015% by moles of the silver halide in the emulsion and adding to the sensitized emulsion at least one palladium salt selected from the group consisting of palladium salts represented by the following general formula:



45 wherein M represents a member selected from the group consisting of an alkali metal atom and an ammonium radical, and X represents a halogen atom selected from the group consisting of chlorine, bromine and iodine atoms, the concentration of said palladium salt in the emulsion being equal to from 0.015 to 0.2% by moles of the silver halide in the emulsion.

14. A process for preparing a high speed photographic silver halide emulsion comprising sensitizing the emulsion with at least one gold compound in a concentration equal to from 0.001 to 0.01% by moles of the silver halide in the emulsion and at least one sulfur sensitizer, and adding to the sensitized emulsion at least one palladium salt selected from the group consisting of palladium salts represented by the following general formulas:



65 wherein M represents a member selected from the group consisting of an alkali metal atom and an ammonium radical, and X represents a halogen atom selected from the group consisting of chlorine, bromine and iodine atoms, the concentration of said palladium salt in the emulsion being equal to from 0.015 to 0.2% by moles of the silver halide in the emulsion.

15. A process for preparing a high speed photographic silver halide emulsion comprising

sensitizing the emulsion by digesting it on the acid side of neutrality in the presence of at least one gold compound in a concentration equal to from 0.001 to 0.01% by moles of the silver halide in the emulsion and at least one sulfur sensitizer, and adding to the sensitized emulsion at least one palladium salt selected from the group consisting of palladium salts represented by the following general formulas:



wherein M represents a member selected from the group consisting of an alkali metal atom and an ammonium radical, and X represents a halogen atom selected from the group consisting of chlorine, bromine and iodine atoms, the con-

centration of said palladium salt in the emulsion being equal to from 0.015 to 0.2% by moles of the silver halide in the emulsion.

ROBERT E. STAUFFER.  
WILLIAM F. SMITH.

## REFERENCES CITED

The following references are of record in the file of this patent:

## UNITED STATES PATENTS

| Number    | Name              | Date          |
|-----------|-------------------|---------------|
| 2,059,642 | Kankelwitz        | Nov. 3, 1936  |
| 2,399,083 | Waller et al.     | Apr. 23, 1946 |
| 2,448,060 | Smith et al.      | Aug. 31, 1948 |
| 2,540,086 | Baldsiefen et al. | Feb. 6, 1951  |